

## UNITED STATES PATENT OFFICE.

GEORGE W. NASH, OF DENVER, COLORADO.

## BRAKE DRESSING COMPOUND AND PROCESS OF MAKING SAME.

No Drawing.

Application filed September 4, 1926. Serial No. 133,727.

This invention relates to a composition for the treatment of the linings of brakes and clutches and to the process of manufacturing the composition.

5 The principal object of the invention is to provide a composition of this character which will increase the wearing qualities of the brake lining, cause the lining to exert a gentle but positive braking effect and to 10 eliminate squeaks, chattering, etc., in brake linings.

Another object of the invention is to provide a composition of this character which will not be injured by water and which 15 will prevent the lining from becoming slick and useless when operating under wet conditions.

20 Still another object is to provide a composition of this character which will clean the brake lining and remove all grease, grit and dirt therefrom.

25 A further object is to provide a composition of this character which will immediately penetrate and saturate the brake lining regardless of its packed or hardened condition.

30 A still further object is to provide a composition of this character which will not evaporate and with which one application will be practically permanent.

I prefer to compound my composition of the following ingredients in substantially the following proportions:

35 1 gallon medium weight motor lubricating oil,  
1 quart kerosene,  
1 ounce powdered or floated mica,  
1 ounce fuller's earth,  
1 ounce bicarbonate of soda,  
40  $\frac{1}{2}$  ounce pumice stone,  
1 ounce glycerine,  
 $\frac{1}{3}$  ounce oil of eucalyptus.

In the composition the motor oil forms 45 the base product. The kerosene cuts or breaks down the motor oil, making an inflammable mixture. The mica acts as a dry lubricant, preventing burning of the brake linings. The fuller's earth is employed as a cleaner and roughener. It acts to microscopically roughen the brake drum and lining, providing a better gripping surface and also acts in combination with the pumice stone to break down or cut the caked grit and dirt from the band and drum, causing 50 this grit and dirt to form in minute rolls and fall from the lining. The bicarbonate

of soda acts as a dryer, that is, it will absorb water or oil which may come in contact with the lining, preventing it from forming a film on the lining, and injuring 60 the gripping qualities thereof. The glycerine is employed as a vehicle for carrying the mica and dispersing it throughout the composition. The oil of eucalyptus is employed for its well known penetrating qualities and 65 assists the entire composition in penetrating the entire depth of the brake lining.

I prefer to manufacture my composition as follows: I mix the soda with the glycerine and in a separate container mix the kerosene with the mica, fuller's earth and pumice stone, the latter mixture being stirred until all solids are in suspension in the kerosene. The motor oil is now heated to the boiling point and the soda and glycerine mixture added thereto. The oil is now kept boiling until the entire mixture has been reduced approximately 1/16th by volume. The kerosene with its contained mica, fuller's earth, and pumice stone is 70 now added and the mixture raised to the "flash point". The vapor from the boiling oil, consisting in the main of kerosene and glycerine vapors, is now ignited and allowed 75 to burn. The boiling and combustion is continued until the mixture is again reduced in volume to approximately 1 gallon. In the reduction the kerosene and glycerine of the compound are burned away, leaving the residue. While the mixture is still warm, 80 but not boiling, the oil of eucalyptus is added. The main purpose in the boiling down of the composition is to vaporize and remove heavy caking greases, such as paraffin, etc., from the mixture. It is the paraffin 85 in lubricating oil that makes it useless for a brake dressing in its natural condition. In the heating the entire glycerine content is not removed, a small amount being retained 90 as a binder for the mica.

100 It is, of course, not necessary to ignite the vapors. They could be allowed to discharge into the atmosphere. The combustion, however, of the vapors assists in heating the surface of the compound to burn out the paraffin. For the lubricating oil refuse crank case oil might be employed after being subjected to a suitable refining process.

105 While I have described in some detail one preferred formula for my composition and a method of carrying out my process, together with the theories which I believe 110

explain the success of the process, it is to be understood that my invention is not limited to the precise formula nor precise procedure described nor is it dependent upon the accuracy of the theories which I have advanced. On the contrary, my invention is not to be regarded as limited except in so far as such limitations are included within the terms of the accompanying claims, in which it is 10 my intention to claim all novelty inherent in my invention as broadly as permissible in view of the prior art.

Having thus described the invention, what I claim and desire secured by Letters Patent is:—

1. A composition for the treatment of brake linings comprising the following ingredients in substantially the named proportions, viz: 1 gallon lubricating oil, 1 ounce powdered mica, 1 ounce fuller's earth, 1 ounce bicarbonate of soda,  $\frac{1}{2}$  ounce pumice stone and  $\frac{1}{3}$  ounce oil of eucalyptus.

2. A composition for the treatment of brake linings which has been formed by 25 the ignition of the ignitable ingredients of the following ingredients in substantially the named proportions, viz: 1 gallon lubricating oil, 1 ounce powdered mica, 1 ounce fuller's earth, 1 ounce bicarbonate of soda,  $\frac{1}{2}$  ounce pumice stone,  $\frac{1}{3}$  ounce oil of eucalyptus, 1 quart kerosene, and 1 ounce glycerine.

3. The process of manufacturing a composition for the treatment of brake linings

comprising heating lubricating oil to the flash point, adding a mixture of kerosene, mica, fuller's earth, and pumice to the boiling oil, igniting the vapors from the boiling oil and continuing the combustion until the mixture has been reduced substantially  $\frac{1}{6}$ th 40 by volume.

4. The process of manufacturing a composition for the treatment of brake linings comprising heating lubricating oil to the flash point, adding a mixture of kerosene, 45 mica, fuller's earth, and pumice to the boiling oil, igniting the vapors from the boiling oil and continuing the combustion until the mixture has been reduced substantially  $\frac{1}{6}$ th by volume and adding oil of eucalyptus to the hot mixture.

5. The process of manufacturing a composition for the treatment of brake linings comprising heating lubricating oil to the flash point, adding a mixture of soda and glycerine to the boiling oil and continuing the boiling until the mixture has been reduced substantially  $\frac{1}{6}$ th by volume, adding a mixture of kerosene, mica, fuller's earth and pumice to the reduced mixture, igniting the vapors from the mixture and continuing the boiling and combustion until the mixture has again been reduced substantially  $\frac{1}{6}$ th by volume.

In testimony whereof, I affix my signature.

GEORGE W. NASH.